

## UNITED STATES PATENT OFFICE.

AUGUSTO PASSALACQUA, OF PARIS, FRANCE.

## PROCESS FOR FACING SHEETS OR OBJECTS OF ALUMINUM AND THE LIKE WITH SHEETS OF HEAVY METAL.

No Drawing.

Application filed December 21, 1923. Serial No. 682,114.

To all whom it may concern:

Be it known that I, AUGUSTO PASSALACQUA, subject of the King of Italy, residing at Paris, France, post-office address 17 Rue du General Brunet, have invented certain new and useful Improvements in Processes for Facing Sheets or Objects of Aluminum and the like with Sheets of Heavy Metal, of which the following is a specification.

- 10 The present invention relates to a process which enables sheets or objects of aluminum or its alloys to be faced or lined with sheets of heavy metal, such as copper, adapted to form a protective layer. The sheets of the protective metal may be exceedingly thin in order to prevent the final product from becoming too heavy whilst at the same time effectively protecting the aluminum.
- 15

20 The advantages of aluminum with a facing of copper should be obvious without being emphasized, in view of the large number of uses to which aluminum thus protected can be put.

25 The sheets of copper or other heavy metal are preferably exceedingly thin, for example some hundredths of a millimetre.

The covering is effected in the following manner:

- 30 The surfaces are first carefully cleaned. The aluminum or the like to be cleaned is first slightly heated to about 100° C., and then a pickling composition prepared in the manner hereinafter described is spread thereupon. The heating of the metal is continued. It first becomes entirely black, and thereupon becomes white as in its normal state.

35 The cleaning composition is produced by mixing together four compositions A—B—C—D, said mixture being effected under certain conditions which will hereinafter be described.

40 Each of the compositions A—B—C—D is composed of a certain number of substances which are specified below.

45 The proportions of the substances herein-  
after specified are merely given by way of example and may actually vary within wide limits without interfering with the cleaning properties of the composition. The propor-  
50 tions may thus be modified without depart-

ing from the spirit and scope of the invention.

## Formula A.

|                                      |     |    |
|--------------------------------------|-----|----|
| Stearic acid                         | 18  | 55 |
| Paraffin                             | 18  |    |
| Resin                                | 18  |    |
| Linseed oil                          | 18  |    |
| Olive oil or generally any other oil | 18  | 60 |
| Lard or analogous fatty substances   | 10  |    |
|                                      | 100 | 65 |

The linseed oil and the olive oil can be replaced by any other analogous oils.

## Formula B.

|                                      | c. c. |    |
|--------------------------------------|-------|----|
| Ordinary or distilled water          | 1,000 | 70 |
| Stannous chloride                    | 60    |    |
| Aluminum sulphate                    | 67    |    |
| Aluminum chloride                    | 82    |    |
| Sodium pyrophosphate                 | 60    | 75 |
| Salammoniac                          | 85    |    |
| 10% aqueous solution of caustic soda | 90    |    |
| Stannous sulphate                    | 55    |    |
| Nitric acid                          | 70    | 80 |
| Zinc chloride                        | 55    |    |
| Potassium cyanide                    | 80    |    |
| Potassium ferrocyanide               | 80    |    |

## Formula C.

|                   |       |    |
|-------------------|-------|----|
| Nickel sulphate   | 75    | 85 |
| Ammonium chloride | 90    |    |
| Citric acid       | 80    |    |
| Distilled water   | 1,000 |    |

## Formula D.

|                      |       |  |
|----------------------|-------|--|
| Stannous chloride    | 80    |  |
| Sodium pyrophosphate | 90    |  |
| Distilled water      | 1,000 |  |

The method of obtaining the cleaning paste used for the tinning will now be described.

First a mixture is made of equal parts or of any other proportions of solutions B—C and D.

Thereupon this mixture is added to the composition A in any suitable proportions,

and the resultant mixture is brought to boiling.

The copper or other heavy metal such as for example lead, may be cleaned in the 5 same way as the aluminum. In order to clean the heavy metals, the ordinary pickling compositions, such as hydrochloric acid, ammonium chloride and the like may also be used.

- 10 The cleaning of the aluminum or its alloys as well as that of the copper or of the other heavy metals may be effected by means of a metallic brush or by any other suitable means.
- 15 As soon as the two pieces, of aluminum on the one hand, and of copper on the other hand, have been thoroughly cleaned, their heating is continued until they reach a temperature which lies between about 300 and 20 550° C., whereupon tin is applied to the surface of the aluminum which is to be faced with the sheet of copper. The copper sheet is thereupon applied to the surface of the aluminum sheet which is coated 25 with tin, and the two pieces thus juxtaposed are subjected to a pressing operation in a hydraulic press or any other suitable press. The pressure is maintained until the metal is almost completely cool.
- 30 On leaving the press the two pieces are united. The tin, used for uniting the aluminum and the copper or other metal or alloys may be employed in the pure state or mixed with other metals melting at a 35 low temperature. The tin may also be entirely replaced by one of these metals or by alloys of these metals. Amongst such metals which are adapted to be added to or substituted for tin, zinc may be men- 40 tioned in the first place.

The above-described cleaning is an operation which becomes more essential with increasing purity of the aluminum used. If the aluminum used is mixed with zinc, 45 this operation becomes less necessary as the proportion of zinc increases. The considerations specified with regard to zinc are obviously also applicable to other impurities in the aluminum.

50 It should be well understood that the process is applicable both to pure metals as well as to their alloys.

Thus the sheet of light metal, instead of 55 consisting of pure aluminum, can consist of alloys of aluminum with lead, tin or the like, or of duralumin and the like.

Moreover, the sheet of protective metal may consist of copper or of other heavy metal alone or alloyed with other metals.

60 The hereinbefore described process enables all receptacles of copper or of other heavy metals used in aviation to be replaced by very light receptacles of aluminum lined with copper. Thus their weight is very considerably lightened, the import-

ance of which increases with the dimensions of the receptacles.

When employing alloys of aluminum which are very resistant, such as for example duralumin, it will be found that an 70 increase in resistance is obtained when comparing a receptacle obtained in accordance with the present process with a receptacle of the same weight consisting entirely of copper. Receptacles produced in accordance with the new process are also more economical than receptacles consisting entirely of copper.

The above considerations applied by way of example to receptacles are also applicable to any other objects manufactured according to the present process.

Whilst the process has hereinbefore been described in connection with the facing of aluminum and its alloys, the same may also 85 be applied to the facing of sheets of other metal.

I claim:—

1. The process for lining objects of light metal with a heavy metal adapted to form 90 a protective layer, which comprises heating the light metal object and the covering sheet of heavy metal, carefully cleaning the surfaces of said pieces to be joined together, continuing heating of the light metal, until it attains a temperature of between 300° C. and 550° C., spreading a metal of a low melting point over the surface of said light metal, superimposing the heated heavy metal sheet upon said spread surface and pressing the two juxtaposed pieces strongly together.

2. The process for lining objects of light metal with a heavy metal adapted to form 105 a protective layer, which comprises heating the light metal object and the covering sheet of heavy metal, carefully cleaning the surfaces of said pieces to be joined together, continuing heating of the light metal, spreading a metal of a low melting point over the surface of said light metal, superimposing the heated heavy metal sheet upon 110 said spread surface, pressing the two juxtaposed pieces strongly together and maintaining the pressure until practically complete cooling of the metallic object.

3. The process for lining objects of aluminum and its alloys with an exceedingly thin coating of heavy metal adapted to form 120 a protective layer, which comprises heating the aluminum object and the covering sheet of heavy metal, carefully cleaning the surfaces of said pieces to be joined together, containing heating of the aluminum-containing piece, spreading a metal of a low melting point over the surface of said aluminum-containing piece, superimposing the heated heavy metal sheet upon said spread surface and pressing the two juxtaposed pieces strongly together.

4. The process for lining objects of aluminum and its alloys with an exceedingly thin coating of heavy metal adapted to form a protective layer, which comprises heating the aluminum-containing object and the covering sheet of heavy metal, carefully cleaning the surfaces of said pieces to be joined together, continuing heating of the aluminum-containing piece, spreading a metal of a low melting point over the surface of said aluminum-containing piece, superimposing the heated heavy metal sheet upon said spread surface, pressing the two juxtaposed pieces strongly together and maintaining the pressure until practically complete cooling of the metallic object. 45
5. The process for lining objects of aluminum and its alloys with an exceedingly thin coating of copper and its alloys adapted to form a protective layer, which comprises heating the aluminum-containing object and the covering sheet of copper-containing metal, carefully cleaning the surfaces of said pieces to be joined together, continuing heating of the aluminum-containing piece, spreading a metal of a low melting point over the surface of said aluminum-containing piece, superimposing the heated copper-containing metal sheet upon said spread surface, pressing the two juxtaposed pieces strongly together and maintaining the pressure until practically complete cooling of the coated object. 50
6. The process for lining objects of aluminum and its alloys with an exceedingly thin coating of copper and its alloys adapted to form a protective layer, which comprises heating the aluminum-containing object and the covering sheet of copper-containing metal, carefully cleaning the surfaces of said pieces to be joined together, continuing heating of the aluminum-containing piece, spreading tin-containing metal over the surface of said aluminum-containing piece, superimposing the heated copper-containing metal sheet upon said spread surface, pressing the two juxtaposed pieces strongly together and maintaining the pressure until practically complete cooling of the coated object. 55
7. A pickling composition, comprising a paste composed of stearic acid, paraffin, resin, linseed oil, olive oil and lard; and a mixture of three aqueous solutions added to said paste and composed of: (1) stannous chloride, aluminum sulphate, aluminum chloride, sodium pyrophosphate, salammoniac, caustic soda, stannous sulphate, nitric acid, zinc chloride, potassium cyanide, and potassium ferrocyanide; (2) nickel sulphate, ammonium chloride, and citric acid; and (3) stannous chloride and sodium pyrophosphate. 60
8. A pickling composition, comprising the following ingredients in substantially the following proportions by weight, viz: a paste composed of 18 parts stearic acid, 18 parts paraffin, 18 parts resin, 18 parts linseed oil, 18 parts olive oil, and 10 parts lard; and a mixture of three solutions composed of: (1) 60 parts stannous chloride, 67 parts aluminum sulphate, 82 parts aluminum chloride, 60 parts sodium pyrophosphate, 85 parts salammoniac, 90 parts of a 10% aqueous solution of caustic soda, 55 parts stannous sulphate, 70 parts nitric acid, 55 parts zinc chloride, 80 parts potassium cyanide, 80 parts potassium ferrocyanide, and 1000 parts water; (2) 75 parts nickel sulphate, 90 parts ammonium chloride, 80 parts citric acid, and 1000 parts water; and (3) 80 parts stannous chloride, 90 parts sodium pyrophosphate, and 1000 parts water. 65
- In testimony whereof I affix my signature. 70
- 75
- 80
- 85

AUGUSTO PASSALACQUA.